

## UNITED STATES PATENT OFFICE

2,336,616

METHOD OF INHIBITING FORMATION OF  
BLACK SPOTS ON TINNED COPPER

Herbert C. Jennison, deceased, late of Fairfield, Conn., by Helen E. Jennison, executrix, Fairfield, Conn., and John C. Bradley, Waterbury, Conn., assignors to The American Brass Company, Waterbury, Conn., a corporation of Connecticut

No Drawing. Application January 16, 1941,  
Serial No. 374,701

8 Claims. (Cl. 204—40)

This invention relates to a method of inhibiting formation of black spots on tinned copper, and this application is a continuation in part of our prior application, Serial No. 189,786, filed February 10, 1938.

For years the dairy machinery industry has used tinned copper for making milk vats, coolers, etc. Tinned copper, that is copper coated with a thin layer of tin, is liked for these articles because it is of comparatively low cost and can be handled and fabricated more easily than the substitutes, such as enamel ware, stainless steel, rich nickel alloys, etc. There is, however, one particularly serious difficulty with tinned copper which is known as black spots or tin pest. It is a serious problem in caring for dairy apparatus. This condition is not due to corrosion of the base metal but rather to an allotropic change in the tin which results in disintegration of the tin coating. Our method prevents or greatly hinders this allotropic change.

It is therefore an object of the present invention to prevent or delay the formation of these black spots, and we have found that this may be done by incorporating a small amount of one or more of certain other metals with the tin. We have found that when a small amount of one or more of the metals of the group consisting of manganese and chromium are deposited with the tin, either simultaneously or successively, the formation of these black spots is materially delayed. It is thought that there is a real alloy formed of tin and other metal or metals at the surface, and that this alloy inhibits the allotropic change in the tin.

As an example when copper was plated by electrodeposition with tin and manganese, manganese sulphate and ammonium sulphate were used. The manganese sulphate was present in the quantity of about 37.5 grams in 125 cc. of water. To this was added 25 cc. of the standard sodium stannate electrolyte of substantially the following solution:

|                  | Grams per liter |
|------------------|-----------------|
| Sodium stannate  | 32              |
| Sodium acetate   | .6              |
| Sodium perborate | .3              |
| Rosin            | .01             |

While this gave good results other solutions might be used. A precipitate which is formed was dissolved with a minimum amount of sulphuric acid, then made neutral with ammonia. The sheet copper while plating was covered with a black spongy deposit which had to be cleaned off every two or three minutes, but underneath

was built up a nice, bright, silvery coating of manganese and tin. Analysis showed that tin and manganese were both present but that the tin greatly predominated with the manganese in relatively small amount. In this case the manganese and tin were simultaneously deposited, but we have also found that the formation of the black spots is hindered or delayed if a coat of commercially pure tin is first put on to the copper and then the tin-manganese coat deposited. Or we can put on the metals separately and in succession, first the layer of tin, then the other metal or metals. Or if desired, we can add to the second coat a third coat of tin or a combination of the tin and the manganese.

As indicated above we have found that chromium when plated in combination with tin in the same manner also prevents or greatly hinders the formation of black spots.

When the copper was plated with chromium the plating was accomplished by depositing alternate layers of chromium and tin, then the copper was heated for an hour in boiling water. For the chromium plating solution any one of a number of good solutions could be used. As an example we used a solution substantially as follows:

|                                          | Grams per liter |
|------------------------------------------|-----------------|
| Chromic acid figured as CrO <sub>3</sub> | 400             |
| Sulphate figured as SO <sub>4</sub>      | 4               |

The plated sheet of copper when tested showed improvement over a pure tin coating in resistance to formation of black spots. Analysis showed chromium and tin present with the tin greatly predominating.

We are not confined to the use of pure metals. The point is that when tin is deposited on the copper in combination with certain other metals the black spot formation is materially hindered. The resultant coating is essentially a tin coating with a small amount of the other metal or metals sufficient in amount to have the effect of inhibiting the allotropic change in the formation of black spots or tin pest. Any amount of the added metal assists in preventing black spot and we prefer not to use more than about ten percent as this has been found to be sufficient.

The coating is put on preferably by a code deposition of the metals from a single electroplating bath, but as suggested above we have also accomplished the desired end by successive deposits from different baths.

We do not wish to fuse the tin coating either in depositing or after it has been deposited. Fusing a tin coating on copper definitely thins

the tin coat by making the tin diffuse into the copper and thus really result in a bronze coating of mostly copper instead of a tin coating or coating mostly tin. In other words subsequent fusing of the tin coating is undesirable in our method for inhibiting black spots as our experiments have indicated it tends to reduce the resistance of the coating to this disease.

Having thus set forth the nature of our invention, what we claim is:

1. A method of inhibiting formation of black spots on tinned copper by contact with liquids, food and beverage products which consists in electrodepositing on the copper a coating of tin and at least one of the metals of the group consisting of manganese and chromium in amount sufficient to inhibit black spot formation and with the resultant coating essentially tin and of at least about 90 per cent of this metal.

2. A method of inhibiting formation of black spots on tinned copper which consists in electrodepositing on the copper a coating essentially tin and metal of the group consisting of manganese and chromium in amount sufficient to inhibit black spot formation and not over about 10 per cent of the resultant coating.

3. A method of inhibiting formation of black spots on tinned copper which consists in electrodepositing on the copper surface a coating consisting essentially of tin and an amount of metal of the group consisting of manganese and chromium sufficient to inhibit black spot formation, and with the resultant coating essentially tin and of at least about 90 per cent of this metal.

4. A method of inhibiting formation of black spots on tinned copper which consists in simultaneously electrodepositing on the copper from a single electroplating bath as a coating tin and another metal from the group consisting of manganese and chromium in amount sufficient to inhibit black spot formation, and with the resultant coating essentially tin and of at least about 90 per cent of this metal.

5. A method of inhibiting formation of black spots on tinned copper which comprises succe- 45

sively electrodepositing on the copper a coating essentially of tin, and other metal from the group consisting of manganese and chromium in amount sufficient to inhibit black spot formation with the resultant coating being at least about 90 per cent tin.

6. A method of inhibiting formation of black spots on tinned copper which consists in the electrical deposition on the copper of a layer of metal by codeposition of tin and metal of the group consisting of manganese and chromium in amount sufficient to inhibit black spot formation from a single electroplating bath, and with the resultant coating essentially tin and of at least about 90 per cent of this metal.

7. An article of manufacture for use in handling food and beverage products, including fabricated vessels, containers or structures made at least partly of copper and an electrodeposited coating on the copper consisting essentially of tin and metal of the group consisting of manganese and chromium in amount sufficient to inhibit black spot formation but not over about 10 per cent of the resultant coating, said coating being on that surface to be used in contact with the food and beverage products whereby the tendency to formation of black spots on the coated copper is inhibited.

8. An article of manufacture for use in handling food and beverage products, including fabricated vessels, containers or structures made at least partly of copper and an electrodeposited alloy coating on the copper consisting essentially of tin and a metal of the group consisting of manganese and chromium in amount sufficient to inhibit black spot formation and with the tin not less than about 90 per cent, said coating being on that surface to be used in contact with the food and beverage products whereby the tendency to formation of black spots on the coated copper is inhibited.

HELEN E. JENNISON,  
*Executrix of Herbert C. Jennison, Deceased.*

JOHN C. BRADLEY.

CERTIFICATE OF CORRECTION.

Patent No. 2,336,616.

December 14, 1943.

HERBERT C. JENNISON, DECEASED, ET AL

It is hereby certified that error appears in the printed specification of the above numbered patent requiring correction as follows: Page 1, second column, line 48-49, for "code deposition" read --co-deposition--; and that the said Letters Patent should be read with this correction therein that the same may conform to the record of the case in the Patent Office.

Signed and sealed this 29th day of February, A. D. 1944.

Leslie Frazer

(Seal)

Acting Commissioner of Patents.